

Feb. 24, 1948.

P. E. HALSTEAD

2,436,644

SPARKING PLUG

Filed April 28, 1944

Fig. 1.



Fig. 2.



INVENTOR

Philip E. Halstead

By Watson, Cole, Brindle & Watson

## UNITED STATES PATENT OFFICE

2,436,644

## SPARKING PLUG

Philip Edward Halstead, Hammersmith, London,  
England, assignor to West Road Co. LimitedApplication April 28, 1944, Serial No. 533,216  
In Great Britain June 11, 1943

1 Claim. (Cl. 123—169)

1

This invention relates to sparking plugs of the kind which incorporate a resistance element as part of the electrical circuit for the purpose of inhibiting electrode erosion and/or suppressing interference with wireless receiving apparatus, and the invention has for its object to provide improvements in the known type of sparking plug wherein an electrode housed within the insulator comprises upper and lower portions having interposed therebetween a resistance element that is in electrical communication with the said upper and lower portions.

In my improved sparking plug the insulator comprises ceramic material and the resistance element comprises ceramic material which is semi-conductive or which is rendered semi-conductive, the resistance element being bonded to the insulator to form an integral part thereof by being fired in situ in the insulator.

The insulator is formed of ceramic material of high electrical resistance and is preferably of the sintered oxide type. It may consist predominantly of aluminium oxide. The resistance element may be formed of ceramic material which is, per se, semi-conductive, or of ceramic material, e. g. clay, which is of high resistivity and which has been rendered semi-conductive by incorporating therewith carbon, metallic carbides or other suitable conducting material or by providing a rod or other formed body of the insulating material with a conducting film or coating, e. g. of platinum or carbon.

The resistance element preferably has a resistance at room temperature of not less than 500 ohms, and the resistance may advantageously be between 1000 and 2000 ohms, say 1500 ohms, where the inhibition of electrode erosion is the main consideration. For the suppression of interference with radio apparatus, it is preferred that the resistance element should have a considerably higher resistance, say 15,000 to 50,000 ohms.

It is preferred that the resistance element and the insulator should have substantially the same coefficients of thermal expansion, for example, the insulator and resistance element may have essentially the same composition. In this manner a very satisfactory seal for the central electrode may be obtained having little or no tendency to fail during use of the plug.

My invention will be further described with reference to the accompanying drawing, in which

Fig. 1 is a central vertical sectional view of one form of insulator assembly in accordance with my invention, and

2

Fig. 2 is a similar view of a modified form of insulator assembly.

Referring first to Fig. 1, the insulator 1 shown therein has a centrally disposed bore 2 and a counterbore 3. The lower portion 4 of the central electrode is housed within bore 2 and has at its upper end a flange which seats on the ledge formed at the junction of bore 2 and counterbore 3. Housed within the lower part of counterbore 10 3 is the resistance element 5, which is bonded to the insulator 1, whilst the upper portion 6 of the central electrode is threaded into the counterbore. The resistance element 5 is in electrical communication with the two portions 4, 6 of the central electrode and in the form of the insulator assembly shown in the drawing a thin layer 7 of silver, graphite or other material of high conductivity is interposed between the resistance element and the adjacent ends of the central electrode sections in order to provide good electrical contact between the resistance element and the electrode sections.

In making the insulator assembly shown in Fig. 1, a finely ground ceramic body mixture having, for example, the composition:

|                                      | Per cent |
|--------------------------------------|----------|
| Al <sub>2</sub> O <sub>3</sub> ----- | 92       |
| SiO <sub>2</sub> -----               | 7        |
| MgO -----                            | 1        |

30 is formed to the shape of the insulator shown in the drawing. After inserting the lower portion 4 of the electrode in the bore 2 of the green body, a small quantity of powdered silver, graphite or other suitable material is placed within the counterbore. Thereafter there is placed within the counterbore the material which is to form the resistance element 5 and which may have the composition:

|                       | Per cent |
|-----------------------|----------|
| Clay -----            | 70       |
| Silicon carbide ----- | 20       |
| Graphite -----        | 10       |

45 A further small quantity of powdered silver, graphite or the like is inserted within the counterbore 3 and the upper portion 6 of the electrode is then screwed into position in counterbore 3. This results in the powdered materials being compressed and consolidated. The assembly thus formed is then fired whereby the material of both the insulator and the resistance element is sintered and matured into a dense non-porous body. At the same time the resistance element 5 is bonded to the insulator 1 thus effectively sealing 50 the bore through the insulator against the pas-

sage of gases and vapours. In a modified method of making the insulator assembly, the insulator and resistance element are formed to shape and fired separately. The components of the insulator assembly are then assembled and the assembly is fired to bond the resistance element to the insulator.

In the modified form of insulator assembly illustrated in Fig. 2, the resistance element comprises a rod 5' of ceramic material, preferably of the same composition as that of the insulator 1, which rod is rendered semi-conductive by a thin peripheral film or layer 8 of platinum, carbon or other conductor of electricity, and the resistance element is bonded to the insulator 1 by a layer of glaze 9 applied to the side of the resistance element. In other respects this assembly is similar to that shown in Fig. 1.

In making the insulator assembly shown in Fig. 2, the insulator 1 and rod 5' may be formed and fired separately. The rod 5' may then be coated all over with a suitable compound which, on heating, will decompose to leave on the rod a thin film of the desired conductor. The rod 5' is then heated to provide the conducting film after which it is coated with a suitable glaze composition. After assembling the coated rod and the electrode sections in the insulator, preferably with a layer of graphite, silver powder or the like interposed between the rod and the electrode sections, the assembly is fired to cause the glaze to bond the resistance element to the insulator.

I claim:

A sparking plug of the kind specified comprising an insulator formed of ceramic material, an electrode housed within the insulator and having upper and lower portions, and a resistance element interposed between said upper and lower portions and in electrical communication therewith, said resistance element comprising a body portion of ceramic material having substantially the same coefficient of thermal expansion as the insulator, said body portion having a coating of conducting material to render the element semi-conductive, and a layer of glaze surrounding said conducting coating, said resistance element being fire bonded to the insulator through said glaze.

PHILIP EDWARD HALSTEAD.

#### REFERENCES CITED

The following references are of record in the file of this patent:

#### UNITED STATES PATENTS

|    | Number    | Name       | Date           |
|----|-----------|------------|----------------|
| 25 | 1,388,373 | Richtmyer  | Aug. 23, 1921  |
|    | 1,745,939 | Loewe      | Feb. 4, 1930   |
|    | 1,927,297 | Rabezzana  | Sept. 19, 1933 |
|    | 1,948,382 | Johnson    | Feb. 20, 1934  |
|    | 1,960,316 | Rabezzana  | May 29, 1934   |
| 30 | 2,301,686 | Doran      | Nov. 10, 1942  |
|    | 2,318,440 | Wall       | May 4, 1943    |
|    | 2,349,432 | Hopps      | May 23, 1944   |
|    | 2,371,211 | Barrington | Mar. 13, 1945  |